

## UNITED STATES PATENT OFFICE

2,074,823

HEAT TREATMENT OF STEEL FOR RESIST-  
ANCE TO CREEPGeorge H. Wright, Ballston Spa, N. Y., assignor  
to General Electric Company, a corporation of  
New YorkNo Drawing. Application September 28, 1934,  
Serial No. 745,853

8 Claims. (Cl. 148—21.5)

The present invention relates to steel which is subjected to relatively high temperatures and more particularly to steel which offers a high resistance to the tendency to increase in length with age, which increase is known generally as "creep", and to a method for making the same.

By the expression "creep value", as employed in the present specification, I mean the number of pounds per square inch which, applied to a material such as steel, will cause it to stretch exactly 1% in 100,000 hours.

In the construction of steam turbines, it is desirable to eliminate or prevent, as far as it is possible to do so, any creep in the shafting or in the fastening means, such as bolts or the like, employed in the construction of such machines. Any creep in these materials results in loss of steam and consequent inefficient operation. Bolts or other fastening means as well as shafting should therefore be employed which not only have the necessary physical characteristics such as tensile strength, elastic limit, elongation and reduction of area but which develop a minimum amount of creep.

Prior to the present invention, it has been substantially impossible to obtain consistently steel having a creep value as high as 20,000 pounds per square inch at temperatures of about 450° C. or higher. It is one of the objects of the present invention to provide steel which not only has a high creep value at temperatures of about 450° C. but which has desirable physical characteristics as well.

In carrying out my invention, steel, which may be a hypo-eutectoid forging, is heated to a temperature above the critical range of the steel and below the point of incipient fusion, for example, about 175° C. or more above the upper critical point and maintained at that temperature for about eight hours, or long enough to eliminate the appearance of any dendrites or banded structure in the steel after cooling. The forging may be brought up to the desired elevated temperature by placing it in a furnace heated at about 300° C. and then slowly increasing the temperature until the desired temperature above the critical range is reached. The time required to heat the forging to this temperature will vary, depending upon the size and character of the forging, but will usually be about one hour per inch of thickness. After the desired temperature is attained, the steel is held at that temperature for about eight hours or long enough to promote diffusion of carbon and to thereby substantially eliminate the appearance of any banded or dendritic structure

after cooling. After the heat treatment the forging may be oil quenched or air cooled, depending upon the size of the forging. For example, forgings of large cross section should in general be oil quenched. In cooling the steel in oil or air, I have found it desirable to cool to a temperature of about 150° C. and then to reheat to a temperature several hundred degrees above room temperature to thereby relieve quenching strains. After reheating, it has been found desirable to again hold the forging in the furnace for a period of time equal to about one hour for each inch of thickness of the forging.

The following is given as an illustration only of the invention.

A forging containing about 0.37% carbon and 1.75% nickel, 0.83% chromium, 0.3% molybdenum with the remainder iron except for incidental impurities, was heated at about 950° C. for eight hours, air cooled, reheated at 650° C. and then cooled in the furnace. As a result of this heat treatment, this forging has a creep value at 450° C. of 33,800 pounds per square inch, and in addition, at room temperature, a tensile strength of 121,000 pounds per square inch, an elastic limit of 80,000 pounds per square inch, an elongation in 2" of 20% and a reduction of area of 58%. The resulting structure obtained by the heat treatment was coarse grained with a structure of uniform appearance.

Steel having the identical composition disclosed above when heated at a temperature of about 825° C., oil quenched and then reheated to about 650° C. and furnace cooled, had a creep value of 22,500 pounds per square inch at 450° C. The tensile strength at room temperature of this second piece of material, after the heat treatment was 140,000 pounds per square inch, the elastic limit 116,000, the elongation in 2" of 22% and the reduction of area 71%.

Steel heated at temperatures in the neighborhood of 950° C. for a period of time sufficient to eliminate the banded appearance after the heat treatment has, as indicated above, great resistance to creep as well as satisfactory physical qualities. Good results also may be obtained by employing an elevated temperature somewhat lower than 950° C. for example about 825° C. provided the forging is quenched or quickly cooled from that temperature. The temperature employed for the draw or reheating may vary considerably and will depend in general upon the physical properties desired in the finished product. As a rule, the temperature of 600° C. to 650° C. will provide satisfactory results.

While the heat treatment here and before set forth provides a steel structure substantially free from bands and having a high creep value, the most satisfactory results will be obtained if 5 the steel to be given the heat treatment is substantially free from dendrites prior to the heat treatment. Under such conditions a steel composition, such as above disclosed, after the heat treatment may have creep values up to about 10 40,000 pounds per square inch at 450° C.

What I claim as new and desire to secure by Letters Patent of the United States is:

1. The method for increasing the resistance of forged hypo-eutectoid steel to creep which comprises heating the steel at temperature at least about 175° C. above its critical range but below the point of incipient fusion for several hours, then quenching the steel.

2. The method for increasing the resistance of forged hypo-eutectoid steel to creep which comprises heating the steel at a temperature at least about 175° C. above its critical range but below the point of incipient fusion for about eight or more hours and air cooling the steel.

25 3. The method for increasing the resistance of forged hypo-eutectoid steel to creep which comprises heating the steel at a temperature at least about 175° C. above its critical range but below the point of incipient fusion for a period of time 30 long enough to eliminate any banded structure after cooling, quenching and then reheating the steel at a lower temperature to thereby remove quenching strains.

4. The method for increasing the resistance of forged hypo-eutectoid steel to creep which comprises heating steel substantially free from

dendrites at a temperature at least about 175° C. above the critical range of the steel but below its point of incipient fusion for a period of time equal to about one hour per inch of thickness of the steel.

5 5. The method for increasing the resistance to creep of forged steel consisting substantially of 0.37% carbon, 1.75% nickel, 0.83% chromium, 0.37% molybdenum, and the remainder iron, which comprises heating the steel to about 950° 10 C. for at least eight hours, quenching and reheating at about 600° C. to 650° C. thereby to relieve quenching strain.

6. The method for increasing the creep resistance of a forged hypo-eutectoid nickel, 15 chrome, molybdenum steel which comprises heating the steel at a temperature of at least 950° C. for at least eight hours, quenching and reheating the steel at about 600° to 650° C.

7. A device, a portion of which is subject to 20 continued stress at elevated temperatures, said portion comprising a forged hypo-eutectoid steel which has been heated for several hours at a temperature in the range between about 175° C. above the critical range of the steel and below its 25 point of incipient fusion.

8. A tension member subject to continued stress at elevated temperatures, said member 30 consisting of a forged hypo-eutectoid nickel, chrome, molybdenum steel which has been heated for at least eight hours at a temperature at least 175° C. above the critical range of the steel but below its point of incipient fusion.

GEORGE H. WRIGHT. 35